

Sept. 12, 1967

SHIRO KIMURA ET AL 3,341,331  
PHOTOGRAPHIC SILVER HALIDE MATERIALS UTILIZING SUCCINMONOAMIDO  
BENZOYL ACETANILIDE COLOR COUPLERS  
Filed March 23, 1964

DYES MADE FROM:

1.  $C_{16}H_{33}CH=CHCHCOHN\text{---}C_6H_4\text{---}COCH_2COHN\text{---}C_6H_4\text{---}COOH$   
 $\text{CH}_2\text{COOH}$   
 $OCH_3$
2.  $C_{16}H_{33}CH=CHCHCOHN\text{---}C_6H_4\text{---}COCH_2COHN\text{---}C_6H_4\text{---}COOH$   
 $\text{CH}_2\text{COOH}$   
 $OC_2H_5$
3.  $C_{17}H_{35}COHN\text{---}C_6H_4\text{---}COCH_2COHN\text{---}C_6H_4\text{---}COOH$   
 $COOH$



INVENTORS

Shiro Kimura  
Makoto Yoshida  
Momotoshi Tsuda

By Stevens, Harris, Miller & Moskow, ATTORNEYS

# United States Patent Office

3,341,331

Patented Sept. 12, 1967

1

3,341,331  
PHOTOGRAPHIC SILVER HALIDE MATERIALS  
UTILIZING SUCCINMONOAMIDO BENZOYL  
ACETANILIDE COLOR COUPLERS

Shiro Kimura, Makoto Yoshida, and Momotoshi Tsuda,  
Kanagawa-ken, Japan, assignors to Fuji Shashin Film  
Kabushiki Kaisha, Kanagawa-ken, Japan, a corporation  
of Japan

Filed Mar. 23, 1964, Ser. No. 354,049  
8 Claims. (Cl. 96—55)

## ABSTRACT OF THE DISCLOSURE

A yellow-forming component or color coupler for silver halide emulsions used in light-sensitive color photography having the following general formula



wherein R is an alkyl group having 8-16 carbon atoms and R' is an alkyl group having 1-4 carbon atoms. The coupler shows a sufficient solubility in aqueous media and a suitable spectral adsorption for color photography.

The present invention relates generally to a photographic sensitive material containing a yellow coupler having the general formula



wherein R is an alkyl group having 8-16 carbon atoms and R' is an alkyl group having 1-4 carbon atoms.

Conventional yellow couplers for a subtractive color process are derivatives of  $\beta$ -keto acid, which have in the molecules at least one carboxyl group or sulfonic acid group as an alkali-soluble group i.e., a group solubilizing the molecule in alkaline media. The alkali-soluble groups of these known derivatives, that is, the carboxyl groups or sulfonic acid groups are ones attached to the benzene nucleus of an anilide or the side chain of a benzoyl nucleus, but most of them are ones attached to the atomic group of one side of an active methylene group.

A coupler which has been used hitherto has a carboxyl group or carboxyl groups but in the known coupler having the carboxyl group or groups at only one side of the active methylene group, the solubility in an alkali of the coupler cannot be improved remarkably by increasing the number of carboxyl groups. Hence, it frequently occurs that the coupler is precipitated when added to an emulsion or even precipitated in an after-treatment step from a photographic sensitive material containing the coupler, which results in reducing markedly the transparency of the image.

Further, when a coupler is used in which at least one carboxyl or sulfonic acid group is introduced into the benzene nucleus of  $\beta$ -keto acid anilide, not only is the absorption spectrum of thus formed pigment shifted to the longer wave length side of the spectrum but also the absorption in green regions of the spectrum is broadened, which adversely affects the color reproduction.

Therefore, an object of this invention is to provide a photographic sensitive material containing a yellow coupler having good solubility.

Another object of this invention is to provide a color

2

photographic sensitive material having good color reproducing property.

A further object of this invention is to provide a color photographic sensitive material which does not have such drawbacks as mentioned above.

The coupler employed in this invention contains hydrophilic carboxyl groups in both groups attached to an active methylene group and has very high solubility in an alkali as compared with a conventional coupler containing one or more alkali-soluble groups in only one of the groups attached to the active methylene group. Therefore, the coupler in this invention is not precipitated when it is added in an emulsion or is not precipitated in an after-treatment step, thereby allowing a color image having excellent transparency to be obtained.

While the absorption spectrum of a pigment shifts always toward the longer wave side of the spectrum when a coupler which contains an electron attractive group such as carboxyl group is used, the absorption spectrum of a pigment does not shift toward the longer wave side and the maximum absorption wave length is narrow when the coupler according to this invention is used. Accordingly, the absorption in the green region which adversely affects the color reproduction is very small when the couplers of this invention are employed.

Moreover, the color image obtained from the coupler according to this invention has a very excellent durability against the effect of temperature, humidity and light.

As described above, a natural color image of excellent color reproduction can be obtained when the couplers according to this invention is used.

Examples of the couplers according to this invention are:

35 (I) 5-carboxy-2-methoxy-(4-octadecenylsuccinmonoamido)benzoyl acetanilide,



(II) 5-carboxy-2-methoxy-(4-tetradecenylsuccinmonoamido)benzoyl acetanilide,



45 (III) 5-carboxy-2-ethoxy-(4-octadecenylsuccinmonoamido)benzoyl acetanilide,



(IV) 5-carboxy-2-methoxy-(3-octadecenylsuccinmonoamido)benzoyl acetanilide,



55 (V) 5-carboxy-2-methoxy-(4-dodecenylsuccinmonoamido)benzoyl acetanilide,





claim 1 wherein said coupler is 5-carboxy-2-methoxy-(4-octadecenylsuccinmonoamido)benzoyl acetanilide.

3. The photographic sensitive material as claimed in claim 1 wherein said coupler is 5-carboxy-2-methoxy-(4-tetradecenylsuccinmonoamido)benzoyl acetanilide.

4. The photographic sensitive material as claimed in claim 1 wherein said coupler is 5-carboxy-2-ethoxy-(4-octadecenylsuccinmonoamido)benzoyl acetanilide.

5. The photographic sensitive material as claimed in claim 1 wherein said coupler is 5-carboxy-2-methoxy-(3-octadecenylsuccinmonoamido)benzoyl acetanilide.

6. The photographic sensitive material as claimed in claim 1 wherein said coupler is 5-carboxy-2-methoxy-(4-dodecenylsuccinmonoamido)benzoyl acetanilide.

7. A light sensitive silver halide photographic emulsion containing a non-diffusing coupler compound of the general formula



10



wherein R is an alkyl group having 8-16 carbon atoms and R' is an alkyl group having 1-4 carbon atoms.

#### References Cited

#### UNITED STATES PATENTS

3,056,674 10/1962 Hoffstadt et al. ----- 96-100

J. TRAVIS BROWN, Primary Examiner.

NORMAN G. TORCHIN, Examiner.

wherein R is an alkyl group having 8-16 carbon atoms and R' is an alkyl group having 1-4 carbon atoms.

8. The process of producing a yellow dyestuff image in a silver halide emulsion which comprises exposing 5 said emulsion to light and developing the same with a primary aromatic amino developer in the presence of a color former for yellow having the general formula

